

# United States Patent [19]

Baldassarri et al.

[11] B 3,925,086

[45] Dec. 9, 1975

[54] **AZOTRIAZOLE AND AZOTETRAZOLE ANTIFOG, ANTISTAIN AND SELECTIVE DESENSITIZERS FOR SILVER HALIDE EMULSIONS**

[75] Inventors: **Agostino Baldassarri, Savona; Luigi Cellone, Albissola Marina-Savona, both of Italy**

[73] Assignee: **Minnesota Mining and Manufacturing Company, St. Paul, Minn.**

[22] Filed: **Mar. 15, 1972**

[21] Appl. No.: **235,011**

[44] Published under the Trial Voluntary Protest Program on January 28, 1975 as document no. B 235,011.

[30] **Foreign Application Priority Data**

Mar. 16, 1971 Italy ..... 49093/71

[52] **U.S. Cl.** ..... 96/109; 96/66.5; 96/56

[51] **Int. Cl.<sup>2</sup>** ..... **G03C 1/34**

[58] **Field of Search** ..... 96/109, 66.5, 66.4, 56; 260/157

[56]

## References Cited

### UNITED STATES PATENTS

|           |         |               |         |
|-----------|---------|---------------|---------|
| 2,453,087 | 11/1948 | Dersch .....  | 96/66.5 |
| 2,588,538 | 3/1952  | Kendall ..... | 96/66.5 |
| 3,563,747 | 2/1971  | Willems ..... | 96/66   |
| 3,615,616 | 10/1971 | Willems ..... | 96/66.5 |
| 3,719,604 | 3/1973  | Prior .....   | 260/157 |

*Primary Examiner*—Norman G. Torchin

*Assistant Examiner*—John L. Goodrow

*Attorney, Agent, or Firm*—Alexander, Sell, Steldt & DeLaHunt

[57]

## ABSTRACT

Azotriazoles and azotetrazoles are effective anti-fogging agents, anti-stain agents and selective desensitizers for silver halide photographic emulsions. Such agents may be employed in reactive association with the emulsions, or in a processing bath prior to or during development of emulsion layers.

12 Claims, No Drawings

**AZOTRIAZOLE AND AZOTETRAZOLE ANTIFOG,  
ANTISTAIN AND SELECTIVE DESENSITIZERS  
FOR SILVER HALIDE EMULSIONS**

The present invention relates to the use of azotriazoles and azotetrazoles as anti-fog, anti-stain and/or selective desensitizers for silver halides photographic emulsions.

Various compounds have long been employed to reduce fog and stain in silver halide emulsions. Certain of these compounds must be contacted with silver halide photographic emulsions in order to effectively inhibit fog; others are desirably employed in processing baths through which silver halide emulsions pass during or prior to development. Certain fog inhibiting compounds in addition tend to desensitize silver halide emulsions. Those desensitizers which desensitize silver halide only to radiation of certain wave lengths, for example, X-rays, are known as "selective" desensitizers, and are particularly useful in silver halide radiographic emulsions.

Many of the compounds which can effectively inhibit fog are unfortunately incapable of similarly inhibiting "stains" (i.e., intense, localized fog centers). Further, certain fog-restraining compounds can be employed only in a silver halide photographic emulsion (U.S. Pat. No. 2,273,152), whereas other compounds can be employed only in photographic processing baths. Moreover, many fog inhibiting compounds do not function as selective desensitizers for silver halide emulsions. It would be highly desirable to provide a single class of compounds capable of restraining fog, restraining "stains", and of selectively desensitizing silver halide emulsions.

It has now been found that azotriazole and azotetrazole compounds are capable of inhibiting fog when placed in contact with a silver halide emulsion (as by being placed in the emulsion, in a layer adjacent the emulsion, or by being placed in a processing bath which is employed prior to or during development of the emulsion). These compounds have also been found to inhibit "stains" in silver halide photographic emulsions, and, in larger quantities, to selectively desensitize silver halide emulsions.

Accordingly, in one embodiment the present invention relates to a silver halide photographic emulsion having contacted therewith at least a fog-inhibiting amount of an azotriazole or an azotetrazole. In another embodiment, the invention relates to a method for inhibiting fog in a silver halide photographic emulsion which comprises contacting the emulsion with an azotetrazole or an azotriazole. In yet another embodiment, the invention relates to an aqueous processing solution for silver halide photographic emulsions adapted for use prior to or during development and containing from about 3 to about 6 milligrams of an azotriazole or an azotetrazole per liter of solution.

The azotriazoles and azotetrazoles of the present invention preferably correspond to the formula



wherein Z and Z' independently represent atoms forming heterocyclic nuclei of the triazole or tetrazole series. By "azotriazole" and "azotetrazole", reference is made to compounds which have respectively two tri-

azole heterocyclic nuclei or two tetrazole heterocyclic nuclei, which nuclei are joined by an  $\text{N}=\text{N}$  linking group through carbon atoms thereof. These compounds may be variously substituted, and it has been found that azotriazoles and azotetrazoles as a class generally exhibit anti-fog, anti-stain and selective desensitization characteristics. In a preferred embodiment, substituents borne by the heterocyclic nuclei of the azotriazoles and azotetrazoles of the invention include hydrogen, alkyl (e.g.,  $\text{C}_1\text{--C}_{20}$  alkyl), alkaline (e.g.,  $\text{C}_1\text{--C}_{20}$ ), and aryl (e.g., phenyl, naphthyl, including substituted aryl such as alkaryl having no more than 15 aliphatic carbon atoms, etc.). Accordingly, in a most preferred embodiment the azotriazoles and azotetrazoles of the present invention correspond to the formula



wherein X is carbon or nitrogen, and each Y group independently represents a hydrogen atom, an alkyl group (e.g.,  $\text{C}_1\text{--C}_{20}$ ), an alkaline group (e.g.,  $\text{C}_1\text{--C}_{20}$ ), or an aryl group (e.g., phenyl, naphthyl, including substituted aryl such as alkaryl containing no more than 20 aliphatic carbon atoms), etc.

In comparison with known fog restrainers, the present invention permits a single class of fog restrainers to be used for many purposes. For example, the triazoles and tetrazoles of the invention are useful both in photographic silver halide emulsions, (e.g., mixed into the emulsion layer or employed in a layer adjacent the emulsion layer) and in photographic processing baths which, for example, are employed either prior to development (as a "pre-bath"), in the developing bath itself, etc. The azotriazole and azotetrazole compounds of the invention are particularly desirable because they are generally readily soluble in common photographic solvents such as water, alcohol, and aqueous alkaline solutions such as developer solutions. It will further be understood that it is most desirable to use highly soluble azotetrazoles or azotriazoles of the invention when they are to be employed in photographic processing baths, and to use the less soluble azotriazoles or azotetrazoles when they are to be used in an emulsion layer or in a layer adjacent an emulsion layer.

The invention may be more easily understood by reference to the following illustrative, non-limiting examples.

**EXAMPLE 1**

5,5'-azotetrazole-1,1'pentahydrate disodium salt



5 g of 5-amino-1H-tetrazole monohydrate (commercial product), (M.P. 103°C) were dissolved into 50 cc of 15% NaOH in a 500 cc flask equipped with mechanical stirrer and reflux apparatus. The solution was brought to the boil, and small amounts of  $\text{KMnO}_4$  (powder) were added, with stirring. After the addition of 6.5 g of  $\text{KMnO}_4$ , the solution became permanently

green. The excess oxidant was eliminated by cautiously adding a few drops of ethanol, and the solution was then rapidly filtered. Upon cooling the intensely yellow colored filtrate, platelets separated and were collected by filtering. 5 g of the product were obtained, corresponding to 67% of the theoretical yield. This compound can be introduced into a photographic emulsion or into a photographic bath in aqueous solution.

| Analysis: | Calculated |      | Found |
|-----------|------------|------|-------|
|           | C%         | H%   |       |
|           | 9.78       | 8.00 |       |
|           | 4.52       | 4.0  |       |

### EXAMPLE 2

#### 5,5'-azotriazole hemihydrate



(prepared according to B. 26 2600 J. Thiele and K. Heidenreich)

8.4 g of 3-amino-1,2,4-triazole (0.1 moles) were dissolved by boiling in 100 cc of H<sub>2</sub>O containing 16 g (0.4 moles) of NaOH in a 300 cc flask equipped with mechanical stirrer and reflux apparatus. 5.4 g of KMnO<sub>4</sub> in powder form were slowly added, with caution, to this solution. The excess oxidant was cautiously eliminated by addition of a few drops of ethanol. The mixture was filtered under vacuum and the yellow liquid obtained was acidified at 15°C with glacial acetic acid. A very fine, pale-yellow powder was separated and collected by filtering and dried under vacuum. Yield: 2 g.

This compound can be usefully introduced into a photographic emulsion or photographic bath in aqueous solutions of sodium carbonate or NaOH.

| Analysis: | Calculated |       | Found |
|-----------|------------|-------|-------|
|           | N%         | C%    |       |
|           | 64.75      | 64.75 |       |
|           | 27.75      | 27.89 |       |
|           | 2.90       | 2.90  |       |

### EXAMPLE 3

#### 3,3'-dimethyl-5,5'-azotriazole



A solution containing 9.8 g of amino-methyl-triazole (0.1 moles) prepared according to B. 26 2599, J. Thiele and K. Heidenreich), 16 g of NaOH (0.4 moles) and 100 cc of H<sub>2</sub>O, was brought to the boil in a 500 cc flask equipped with mechanical stirrer and reflux apparatus. Powdered KMnO<sub>4</sub> was cautiously added in small amounts until the solution became permanently green

(5.5 g of potassium permanganate). The excess oxidant was eliminated by addition of a few drops of ethanol. The separated brown manganese dioxide was filtered under vacuum. The cooled yellow solution was acidified (*t* = 15°C) with glacial acetic acid. A sulfur-yellow, very fine powder separated out and was filtered, dissolved in NH<sub>4</sub>OH, precipitated with CO<sub>2</sub> and washed with H<sub>2</sub>O. Yield: 2 g.

This compound can be usefully introduced into an emulsion or photographic bath in solutions of sodium carbonate or NaOH.

| Analysis: | Calculated |       | Found |
|-----------|------------|-------|-------|
|           | N%         | C%    |       |
|           | 58.33      | 57.94 |       |
|           | 37.50      | 37.23 |       |
|           | 4.20       | 4.31  |       |

### EXAMPLE 4

#### 1,1'-diphenyl-5,5'-azotetrazole



(prepared according to Journ. Prakt. 2, 134 282, R. Stolle).

20 g of 1-phenyl-5-amino-tetrazole (prepared according to C.A. 65 20137h, C.D. Bassinger and Takanishi Enkoji) were dissolved in 500 cc of boiling water in a 2 liter flask equipped with a mechanical stirrer and reflux apparatus. Gaseous chlorine was passed through the boiling solution. After a few minutes an orange colored solid began to separate. After about 4 hours it was noticed that a further addition of chlorine did not cause separation of more solid. The solid was collected by hot filtration, washed with 500 cc of cold water and dried with air. Yield: 15 g. After crystallization of the product from 1500 cc of boiling glacial acetic acid, 12.5 g of felted orange needles, M.P. 227°C. were obtained.

This compound can be usefully introduced into a photographic silver halide emulsion or into a photographic bath in ethanol of dimethylformamide solution.

| Analysis: | Calculated |       | Found |
|-----------|------------|-------|-------|
|           | C%         | H%    |       |
|           | 52.78      | 52.59 |       |
|           | 3.14       | 3.17  |       |
|           | 43.98      | 43.83 |       |

### EXAMPLE 5

#### 1,1'-dimethyl-5,5'-azotetrazole



(prepared according to J. Phys. Chem. 61, 265, M. M. Williams, W. S. McEwan and R. A. Henry).

20 g of 1-methyl-5-azotetrazole, prepared according to J.A.C.S. 76 923, R. A. Henry and W. G. Finnegan, were suspended in 100 cc of water. 100 cc of a 10% ac-

tive chlorine sodium hypochlorite solution were added. The mixture was brought to the boil and maintained for 15 minutes at this temperature. The resulting solution was allowed to cool in ice and was kept at 0°C overnight. The yellowish solid which separated was filtered under vacuum, washed with water and dried under vacuum. Yield: 8 g. The product obtained was crystallized from 60 cc of boiling ethyl acetate. A yellow powder (6.2 g., M.P. 120°-122°C) which according to the literature corresponds to a mixture of the "cis" and "trans" forms, was obtained.

10 This compound can be usefully introduced into emulsions or photographic baths in ethanol solution.

| Analysis: | Calculated | Found |
|-----------|------------|-------|
| C%        | 24.72      | 25.12 |
| H%        | 3.05       | 3.37  |
| N%        | 72.10      | 70.98 |

#### EXAMPLE 6

##### 2,2'-dimethyl-5,5'-azotetrazole



10 g of 2-methyl-5-amino-tetrazole, suspended into 50 cc of H<sub>2</sub>O were added to 50 cc of a 10% active chlorine sodium hypochlorite solution. An exothermic reaction occurred and the mixture became orange in color. The mixture was brought to the boil for 20 minutes, and was then cooled in ice. After two hours the separated crystalline, orange-yellow solid (5.5 g.) was filtered off and crystallized from 45 cc of acetyl acetate. 4 g of orange needles, M.P. 170°-173°C were obtained.

15 This compound can be usefully introduced into emulsions or photographic baths in ethanol solution.

| Analysis: | Calculated | Found |
|-----------|------------|-------|
| C%        | 24.72      | 24.94 |
| H%        | 3.09       | 3.31  |
| N%        | 72.10      | 71.42 |

#### EXAMPLE 7

##### 1,1'-diallyl-5,5'-azotetrazole



6.25 g of 1-allyl-5-amino-tetrazole (prepared according to J.A.C.S. 76, 923, R. A. Henry and W. G. Finnegan) were dissolved in 100 cc of water in a 500 cc flask equipped with a stirrer, reflux and dropping funnel. While the solution was maintained at the boil, 0.1 moles of sodium hypochlorite (in a 8.5% active chlorine solution) were added over a period of 10 minutes with vigorous stirring. The mixture was allowed to cool slowly to room temperature, and was then filtered under vacuum. The orange solid which was obtained

was washed with 100 cc of water and dried at 30°C under vacuum. Yield: 5 g. M.P. 100°C.

This compound can be usefully introduced into emulsions or photographic baths in ethanol solution.

| Analysis: | Calculated |      | Found |
|-----------|------------|------|-------|
|           | C%         | H%   | N%    |
|           | 38.99      | 4.06 | 56.85 |
|           | 38.49      | 4.31 | 56.25 |

#### EXAMPLE 8

##### 2,2'-diallyl-5,5'-azotetrazole



25 3.13 g (0.025 moles) of 2-allyl-5-amino tetrazole dissolved in 50 cc of boiling water, were combined during a 10 minute period with stirring with 0.05 moles of sodium hypochlorite in a 8.5% active chlorine solution while keeping the mixture at boiling point. A crystalline yellow solid began immediately to separate. The mixture was rapidly cooled to 0°C, filtered under vacuum, and washed with 50 cc of cold water. The residue was dried at 30°C under vacuum. 2.5 g of product were obtained, which were then dissolved in 45 cc of ethyl acetate. 30 The solvent was then concentrated to 15 cc and allowed to crystallize. 1.5 g of orange-yellow small needles, M.P. 94°-96°C were obtained.

35 This compound can usefully be introduced into emulsions or photographic baths in ethanol solution.

| Analysis: | Calculated |      | Found |
|-----------|------------|------|-------|
|           | C%         | H%   | N%    |
|           | 38.49      | 4.06 | 56.89 |
|           | 38.42      | 4.21 | 56.28 |

#### EXAMPLE 9

For the compounds of example 1 to 8 and for the 5,5'-dichloro-2,2'-azopyrine (compound C), suitable 50 solvents have been selected, and the solubility of these compounds at 20°C in these solvents has been determined. The results are reported in the following table 1.

Table I

| Compound | Solvent          | Solubility (weight %) |
|----------|------------------|-----------------------|
| C        | Ethanol          | 0.0009                |
| 1        | Water            | 10                    |
| 2        | 2% NaOH in water | 10                    |
| 3        | 2% NaOH in water | 10                    |
| 4        | Ethanol          | 0.5                   |
| 5        | Ethanol          | 0.5                   |
| 6        | Ethanol          | 0.5                   |
| 7        | Ethanol          | 1                     |
| 8        | Ethanol          | 1                     |

#### EXAMPLE 10

A high-sensitivity, physically seasoned, washed, and chemically sensitized silver bromo-iodide emulsion, containing 98.2 moles of bromide and 1.8 moles of io-

dide percent of halide, was divided in several portions to which were added respectively 1-phenyl-5-mercaptop-tetrazole (labeled A), 5-methyl-benzotriazole (labeled B), and the compounds of Examples 1 to 8.

Each single portion was spread on a cellulose triacetate support and covered with a protective gelatin

from a tungsten lamp, were developed at 20°C in the respective developer portions for 3 minutes, 6 minutes and 12 minutes. The results of a densitometer reading of the developed samples are reported in table 3.

Table 3

| Developer                           | Relative Sensitivity |       |        | Fog   |       |        |
|-------------------------------------|----------------------|-------|--------|-------|-------|--------|
|                                     | 3 min                | 6 min | 12 min | 3 min | 6 min | 12 min |
| Control                             | 100                  | 95    | 90     | 0.28  | 0.34  | 0.45   |
| Control + compound of Example No. 2 | 60                   | 73    | 73     | 0.17  | 0.18  | 0.21   |

layer. Each of the resulting samples was exposed to light from a tungsten lamp and developed for 3 minutes at 20°C in a developer of the following composition:

|                          |      |
|--------------------------|------|
| Metol                    | 3 g  |
| Anhydrous sodium sulfite | 50 g |
| Hydroquinone             | 9 g  |

Example 11 was repeated except that photographic samples of a semi-ammoniacal, high sensitivity, silver 20 bromo-iodide emulsion, containing 98 mole % bromide and 2 mole % iodide were employed. Densitometry results are reported in table 4.

Table 4

| Developer                           | Relative Sensitivity |       |       | Fog   |       |        |
|-------------------------------------|----------------------|-------|-------|-------|-------|--------|
|                                     | 3 min                | 6 min | 2 min | 3 min | 6 min | 12 min |
| Control                             | 105                  | 98    | 95    | 0.18  | 0.25  | 0.36   |
| Control + compound of Example No. 2 | 68                   | 76    | 75    | 0.13  | 0.15  | 0.18   |

|                            |         |
|----------------------------|---------|
| Anhydrous sodium carbonate | 50 g    |
| Potassium bromide          | 3 g     |
| Water to                   | 1000 cc |

Densitometry results for the thus processed samples are reported in table 2.

Table 2

| Compound | $\mu\text{M}/\text{MA}$ g | Relative Sensitivity | Fog  |
|----------|---------------------------|----------------------|------|
| Blank    | —                         | 100                  | 0.28 |
| A        | 1                         | 100                  | 0.28 |
| A        | 10                        | 100                  | 0.28 |
| A        | $10^2$                    | 105                  | 0.28 |
| A        | $10^3$                    | 16                   | 0.22 |
| B        | 1                         | 100                  | 0.28 |
| B        | 10                        | 100                  | 0.28 |
| B        | $10^2$                    | 95                   | 0.28 |
| B        | $10^3$                    | 79                   | 0.29 |
| I        | 1.25                      | 89                   | 0.18 |
| I        | 2.5                       | 56                   | 0.15 |
| I        | 5                         | 45                   | 0.12 |
| 2        | $5 \cdot 10^{-1}$         | 89                   | 0.19 |
| 2        | 1                         | 71                   | 0.18 |
| 2        | 2.5                       | 50                   | 0.16 |
| 3        | $5 \cdot 10^{-1}$         | 85                   | 0.18 |
| 3        | 1                         | 75                   | 0.17 |
| 4        | 2.10                      | 100                  | 0.21 |
| 4        | $10^2$                    | 66                   | 0.16 |
| 4        | $5 \cdot 10^2$            | 63                   | 0.13 |
| 5        | $2 \cdot 10^{-1}$         | 75                   | 0.20 |
| 5        | $5 \cdot 10^{-1}$         | 50                   | 0.18 |
| 5        | 10                        | 25                   | 0.14 |
| 6        | 2.10                      | 100                  | 0.21 |
| 6        | $10^2$                    | 84                   | 0.15 |
| 6        | $5 \cdot 10^2$            | 56                   | 0.10 |
| 7        | 5.10                      | 100                  | 0.20 |
| 8        | $10^2$                    | 89                   | 0.25 |

35 3M Medical X-Ray Film, Type R, was exposed to blue light from a tungsten lamp and was divided into two portions. One portion was developed for 30 minutes at 30°C in the following developer.

40 Anhydrous sodium sulfite 2 g  
2-amino-5-N,N-ethyl- $\beta$ -methan-sulfonamido-ethyl-toluene  
sulfonate 5.5 g  
Dihydrate sodium metaborate 60 g  
Sodium bromide 1.6 g  
Water to 1000 cc

45 The remaining portion was identically developed in an identical developer which, however, additionally contained 200  $\mu\text{M}$  per liter of the compound of Example 2.

50 The results of a densitometer reading of the developed samples are reported in table 5.

Table 5

|  | Relative Sensitivity |                                 | Fog  |
|--|----------------------|---------------------------------|------|
|  | Control              | Control + compound of Example 2 |      |
|  | 100                  | 120                             | 0.23 |
|  |                      |                                 | 0.03 |

EXAMPLE 11

65 A quantity of the developer of Example 10 was divided into two portions. To one portion was added 50  $\mu\text{M}$  of the compound of Example 2. Samples of the photographic material of Example 10, exposed to light

Photographic material similar to that of Example 10 was exposed to the light from a tungsten lamp and divided into three samples. One sample was developed in a developer of the following formula:

EXAMPLE 14

|                            |         |
|----------------------------|---------|
| Metol                      | 3 g     |
| Anhydrous sodium sulfite   | 50 g    |
| Hydroquinone               | 9 g     |
| Glutaraldehyde bisulfite   | 13 g    |
| Anhydrous sodium carbonate | 50 g    |
| Potassium bromide          | 3 g     |
| Water to                   | 1000 cc |

The second and third samples were identically developed, except that the developers for these samples contained respectively 50  $\mu$ M per liter of the compounds of Examples 2 and 3.

Results of densitometer readings are reported in table 6.

Table 6

|                                 | Relative Sensitivity | Fog  |
|---------------------------------|----------------------|------|
| Control                         | 100                  | 0.75 |
| Control + compound of Example 2 | 160                  | 0.21 |
| Control + compound of Example 3 | 140                  | 0.10 |

## EXAMPLE 15

A sheet of 3M Medical X-Ray Film Type R was exposed to blue light from a tungsten lamp and was divided into two portions. One portion was developed for 30 minutes at 35°C in the following developer:

|                            |         |
|----------------------------|---------|
| Potassium metabisulfite    | 42.0 g  |
| Potassium hydroxide        | 47.0 g  |
| Hydroquinone               | 30.0 g  |
| Phenidone                  | 1.4 g   |
| Glutaraldehyde             | 5.0 g   |
| Potassium bromide          | 3.9 g   |
| Water to                   | 1000 cc |
| Acetic acid to a pH = 10.1 |         |

The second sample was identically developed except that the developer containing 200  $\mu$ M per liter of the compound of Example 2.

Results of densitometer readings are reported in table 7.

Table 7

|                                     | Relative Sensitivity | Fog  |
|-------------------------------------|----------------------|------|
| Control                             | 100                  | 0.85 |
| Control + compound of Example No. 2 | 100                  | 0.45 |

## EXAMPLE 16

To samples of a medium sensitivity, physically seasoned, washed and chemically sensitized silver bromo-iodide emulsion containing 97.5 moles % of bromide and 2.5 mole % of iodide, were added various amounts of compounds of the present invention, of red mercury iodide (a known selective desensitizer), and of 1-phenyl-5-mercaptopentetrazole (labeled A).

The resulting emulsions were then spread on cellulose triacetate supports, and samples of the corresponding materials were exposed to white light and to X-rays of various energy. The exposed samples were then developed for 3 minutes at 20°C in the developer of Example 10.

Densitometry results are reported in table 8.

## 10

Table 8

| Compound         | $\mu$ M/MA g        | White light | Relative Sensitivity<br>R X<br>67 K V | Relative Sensitivity<br>R X<br>200 K V | Fog  |
|------------------|---------------------|-------------|---------------------------------------|----------------------------------------|------|
| —                | —                   | 100         | 100                                   | 100                                    | 0.27 |
| HgI <sub>2</sub> | 0.5                 | 71          | 100                                   | 90                                     | 0.25 |
| HgI <sub>2</sub> | 1.0                 | 55          | 90                                    | 75                                     | 0.20 |
| HgI <sub>2</sub> | 2.5                 | 27          | 56                                    | 45                                     | 0.10 |
| HgI <sub>2</sub> | 5.0                 | 15          | 30                                    | 30                                     | 0.04 |
| A                | 1.0                 | 100         | 100                                   | 100                                    | 0.27 |
| A                | 10.0                | 100         | 100                                   | 79                                     | 0.27 |
| A                | 5.10                | 50          | 70                                    | 60                                     | 0.24 |
| A                | 10 <sup>2</sup>     | 25          | 50                                    | 50                                     | 0.22 |
| 1                | 5.0                 | 71          | 100                                   | 100                                    | 0.17 |
| 1                | 10                  | 40          | 100                                   | 90                                     | 0.16 |
| 1                | 10 <sup>2</sup>     | 31          | 100                                   | 83                                     | 0.08 |
| 1                | 5.10 <sup>2</sup>   | 5           | 50                                    | 38                                     | 0.04 |
| 2                | 5.10                | 50          | 89                                    | 89                                     | 0.10 |
| 2                | 10 <sup>2</sup>     | 25          | 70                                    | 70                                     | 0.08 |
| 2                | 2.5.10 <sup>2</sup> | 5           | 50                                    | 40                                     | 0.04 |
| 3                | 10                  | 71          | 105                                   | 100                                    | 0.06 |
| 3                | 10 <sup>2</sup>     | 45          | 100                                   | 71                                     | 0.06 |
| 3                | 2.5.10 <sup>3</sup> | 10          | 71                                    | 50                                     | 0.04 |
| 6                | 10 <sup>3</sup>     | 63          | 105                                   | 100                                    | 0.08 |
| 6                | 10 <sup>4</sup>     | 31          | 89                                    | 89                                     | 0.04 |
| 7                | 10 <sup>3</sup>     | 50          | 100                                   | 89                                     | 0.08 |
| 7                | 10 <sup>4</sup>     | 31          | 89                                    | 89                                     | 0.04 |
| 8                | 2.5.10 <sup>3</sup> | 25          | 63                                    | 25                                     | 0.13 |

## 25

## EXAMPLE 17

A cellulose triacetate support was thinly coated with gelatin containing powdered iron. Three samples of the resulting material, drawn at random, were each divided into four parts. On the first part a high sensitivity, silver bromo-iodide containing 98 moles % of bromide and 2 mole % of iodide were coated. On the other three parts of each sample, the same emulsion to which had been added respectively the compounds of Examples 1 and 2 and the 1-phenyl-5-mercaptopentetrazole (labeled A) were coated. On each element thus obtained a protective gelatin layer was coated. The resulting elements were kept 10 minutes in a cold state and were then developed 10 minutes at 20°C in the developer of Example 10. The white and black points on each of the resulting elements were counted.

The results are given in table 9.

Table 9

| Compound | $\mu$ M/MA g    | No. of Points<br>Sample 1 | No. of Points<br>Sample 2 | No. of Points<br>Sample 3 |
|----------|-----------------|---------------------------|---------------------------|---------------------------|
| —        | —               | 150                       | 103                       | 89                        |
| A        | 10 <sup>3</sup> | 145                       | 102                       | 91                        |
| Ex. 1    | 1.5             | 15                        | 17                        | 7                         |
| Ex. 2    | 0.5             | 20                        | 30                        | 15                        |

## 45

## EXAMPLE 18

A high-sensitivity, physically seasoned, washed and chemically sensitized silver bromo-iodide emulsion containing 98.5 mole % of bromide and 1.5 mole % of iodide was divided into two parts. To one part was added chrome alum, and to the other part, in addition to the chrome alum, was added the compound of Example 2. Each part was then spread on a polyester support and was covered by a protective gelatin layer. Samples of each part were exposed to the light of a tungsten lamp and were mechanically developed in a bath of the following composition:

|                          |        |
|--------------------------|--------|
| Phenidone                | 0.3 g  |
| Anhydrous sodium sulfite | 50.0 g |
| Hydroquinone             | 9.0 g  |

## 50

## -continued

|                            |         |
|----------------------------|---------|
| Glutaraldehyde bisulfite   | 13.0 g  |
| Anhydrous sodium carbonate | 50.0 g  |
| Potassium bromide          | 3.0 g   |
| Water to                   | 1000 cc |

According to the time and temperature indicated in table 10 below.

The developed material was fixed in a bath of the following composition:

|                                 |         |
|---------------------------------|---------|
| Anhydrous sodium sulfite        | 50.0 g  |
| Pentahydrate sodium thiosulfate | 400.0 g |
| Glutaraldehyde bisulfite        | 13.0 g  |
| Water to                        | 1000 cc |

and washed for a total processing time of 90 seconds. Densitometer readings are reported in table 10.

Table 10

| Compound | $\mu\text{M}/\text{MAG}$ | Developing bath temperature | Developing Time | Relative Sensitivity | Fog  |
|----------|--------------------------|-----------------------------|-----------------|----------------------|------|
| Control  | —                        | 35°C                        | 23 sec.         | 100                  | 0.26 |
| Ex. 2    | $6.25 \cdot 10^{-1}$     | 35°C                        | 23 sec.         | 89                   | 0.14 |
| Control  | —                        | 37.8°C                      | 23 sec.         | 112                  | 0.38 |
| Ex. 2    | $6.25 \cdot 10^{-1}$     | 37.8°C                      | 23 sec.         | 93                   | 0.26 |
| Control  | —                        | 40.6°C                      | 23 sec.         | 112                  | 0.56 |
| Ex. 2    | $6.25 \cdot 10^{-1}$     | 40.6°C                      | 23 sec.         | 102                  | 0.38 |

The silver halide photographic emulsions of the present invention are silver chloride, silver bromide and silver iodide emulsions and mixtures thereof such as for example, silver bromoiodide and silver chlorobromide iodide. Such emulsions may include synthetic polymeric gelatin substitutes or additives, such as dextrane, polyvinyl alcohol, polyvinyl pyrrolidone, partially hydrolyzed polyvinyl acetate, polyethylacrylate, polymethylmethacrylate, polyamides, etc. The emulsions of the invention may be chemically sensitized with naturally active gelatin, by addition of chemical sensitizers such as thiourea, allylthiourea, thiocyanates, thiosulfates, etc. Sensitization may be effected by the addition of noble metals, such as gold salts. Spectral sensitizers may be employed in emulsions of the invention, such as cyanine and merocyanine dyes. Moreover, the emulsions of the invention may include such additives as color couplers, filtering dyes, surfactants, hardeners, stabilizers, additional fog-restrainers, plasticizers, oxidizing agents, developing accelerators, etc. To form a photographic element, the emulsions of the invention may be coated upon any convenient support such as polyester, cellulose acetate, and the like.

The azotriazoles and azotetrazoles of the invention may be conveniently introduced in the form of solutions into emulsions during preparation thereof. Although it is generally preferred to incorporate the azotriazole and azotetrazole compounds of the invention directly into emulsion layers, these compounds may also be incorporated into layers adjacent the emulsion layers so that the silver halide emulsions are in contact therewith. As antifog and antistain agents, the azotriazoles and azotetrazoles of the invention are preferably used in amounts ranging from about 0.03 mg. to

about 0.2 mg. per kilogram of emulsion, and as selective desensitizers these compounds are preferably used in amounts ranging from 3 to 60 mg. per kilogram of emulsion.

The processing baths of the present invention, as noted previously, may be photographic "pre-baths", such as those known to the art to be useful prior to treatment of a photographic emulsion with a developing solution. Predevelopment baths usually (but not necessarily) are acidic and may contain hardeners such as aldehydes and the like. The azotriazole and azotetrazole compounds of the invention may, of course, also be employed in developing baths. Such baths are normally alkaline and include one or more silver halide photographic developing agents such as hydroquinone, metol, metol-hydroquinone, phenidone, hydroquinone-phenidone, and various p-phenylene diamine materials,

the latter being useful in color development processes. The processing baths of the invention (pre-baths and developer baths) preferably employ from 3 to about 60 milligrams of azotriazole or azotetrazole compound per liter of solution.

What we claim is:

1. A silver halide photographic emulsion having contacted therewith at least a fog-inhibiting amount of an azotriazole or an azotetrazole.
2. The emulsion of claim 1 wherein said anti-fogging agent is a 5,5'-azotetrazole-1,1'-disodium salt.
3. The emulsion of claim 1 wherein said anti-fogging agent is a 5,5'-azotriazole.
4. The emulsion of claim 1 wherein said anti-fogging agent is a 3,3'-dimethyl-5,5'-azotriazole.
5. The emulsion of claim 1 wherein said anti-fogging agent is a 1,1'-diphenyl-5,5'-azotetrazole.
6. The emulsion of claim 1 wherein said anti-fogging agent is a 1,1'-dimethyl-5,5'-azotetrazole.
7. The emulsion of claim 1 wherein said anti-fogging agent is a 2,2'-dimethyl-5,5'-azotetrazole.
8. The emulsion of claim 1 wherein said anti-fogging agent is a 1,1'-diallyl-5,5'-azotetrazole.
9. The emulsion of claim 1 wherein said anti-fogging agent is a 2,2'-diallyl-5,5'-azotetrazole.
10. A method for inhibiting fog in a silver halide photographic emulsion which comprises contacting said emulsion with an azotetrazole or an azotriazole.
11. A method for inhibiting fog and stain in a silver halide emulsion which comprises contacting said emulsion with an azotriazole or an azotetrazole.
12. The emulsion of claim 1 wherein there is a fog-inhibiting amount of azotriazole contacted therewith.

\* \* \* \* \*